

1

2,839,394

## MAGNESIUM ALLOYS

Rene Lucien, Paris, and Emile Tetart, Louvie-Juzon, France, assignors to Societe d'Inventions Aeronautiques et Mecaniques S. I. A. M., Fribourg, Switzerland, a corporation of Switzerland

No Drawing. Application May 26, 1954  
Serial No. 432,576

Claims priority, application France November 9, 1953

## 2 Claims. (Cl. 75—168)

Alloys of the group magnesium-zinc or magnesium-zinc-manganese are already well known in which cerium is incorporated, either in the pure state or in the form of "mischmetall" (rare earths) so as to make them less subject to micro-porosity. The alloys obtained in this way are, however, extremely difficult to prepare; they are indeed very oxidisable, very inclined to form a coarse crystallisation, and finally they are very sensitive to the proportion of the silicon content of the alloy. On the other hand, the problem of micro-porosity cannot be resolved for these alloys other than by a compromise, since a choice must be made between very good mechanical characteristics accompanied by micro-porosity (having a high zinc content and a low content of mischmetall), or on the other hand, an absence of micro-porosity which is accompanied by low mechanical characteristics (a low zinc content and a high content of mischmetall).

The applicants decided to obtain alloys which, as far as possible, were free from all these various drawbacks. To this end, they studied in a systematic manner the specific effect on these alloys of the main rare earths applied to them one by one, while at the same time taking advantage of the known useful properties obtained by the presence of beryllium, that is to say in contributing, to a large extent, to the avoidance of the detrimental effects of oxidation while hot.

In these circumstances, the applicants have found that among the rare earths which are usable on an industrial scale, lanthanum in the practically pure state (which means that it is present in a proportion of more than 90% in a rare earth) gives the most favourable results in avoiding or reducing micro-porosity.

In accordance with the present invention, use is made of practically pure lanthanum in a content which is preferably of the order of 0.5 to 1.5%. It has been found in particular that a 6% zinc alloy containing lanthanum is practically free from micro-porosity.

A particular alloy of magnesium which conforms with the invention has the following composition:

|                             |                              |
|-----------------------------|------------------------------|
| Zinc                        | 6 to 7%.                     |
| Lanthanum, practically pure | 0.5 to 1.5%, for preference. |
| Aluminium                   | 0.5% for preference.         |
| Beryllium                   | 0.01%.                       |
| Silicon                     | Admissible up to 0.15%.      |
| Magnesium                   | The remainder.               |

The presence of the aluminium facilitates the addition of the glucinum to the alloy and in association with it, gives the alloy important casting properties.

In all the above-mentioned alloys, the lanthanum which is referred to as practically pure, is intended to include, in particular, rare earths containing about 92% of lanthanum with 4% of neodymium and 4% of praseodymium.

The mechanical characteristics of the alloys such as defined above are, however, slightly lower than with the

2

other rare earths under the normal conditions of preparation, when the content of zinc is low which requires that the zinc content be maintained between 6 and 7%.

In this connection, the applicants have found that, among the rare earths, the choice of didymium to the extent of a preferred content of 0.5 to 2% of didymium results in better mechanical characteristics. It is necessary that the didymium should contain less than 10% of lanthanum and that it should be practically free from cerium.

The addition of didymium made in accordance with these conditions to the alloys magnesium-zinc-aluminium (0.5%)—beryllium (0.01%), enables high mechanical characteristics to be obtained, even in cases where the zinc content is low and the didymium content is high, for example 1.5%.

A particular alloy which has these characteristics may have the following composition:

|           |                         |
|-----------|-------------------------|
| Zinc      | 5 to 7%.                |
| Didymium  | 0.5 to 2%.              |
| Aluminium | 0.5% for preference.    |
| Beryllium | 0.01%.                  |
| Silicon   | Admissible up to 0.15%. |
| Magnesium | The remainder.          |

It will be observed that the presence of silicon may be admitted in the alloys according to the invention up to a limiting content which is about ten times greater than the safe limit which could have been permitted in the case of previous alloys, if acceptable mechanical characteristics were to be obtained.

Finally, it will be seen that the advantageous results accruing from the use of didymium enable the elimination of the usual dilemma, referred to at the beginning of this specification, in the case of the group of alloys magnesium-zinc-mischmetall.

The invention especially includes alloys which conform to these characteristics and in which the didymium used with a preferred content of 0.5 to 2% has the following composition:

|              | Percent  |
|--------------|----------|
| Neodymium    | 60 to 75 |
| Praseodymium | 10 to 15 |
| Samarium     | 16 to 17 |
| Lanthanum    | 0. to 10 |
| Cerium       | 0        |

The invention also comprises a heat treatment applied to the alloys which have the characteristics referred to above.

Homogenisation is carried out in two temperature stages, the first at about 338° C. and the second at a temperature in the vicinity of 460° C. By this means, increase of grain size during heat treatment is avoided. For hardening, simple cooling in air is sufficient. This homogenising treatment is followed by a tempering process which is also carried out in two temperature stages, for example, the first stage at 140° C. and the second at 160° C. These tempering temperatures can, however, be varied between fairly wide limits; for the first stage between 120° and 150° C., and for the second stage between 140° and 200° C. depending on the results it is desired to obtain and the composition of the alloy.

What we claim is:

1. Magnesium alloys of the group comprising magnesium, zinc, aluminium, glucinum, the said alloys having the following composition:

|                             |                  |
|-----------------------------|------------------|
| Zinc                        | 6 to 7%.         |
| Lanthanum, practically pure | 0.5 to 1.5%.     |
| Aluminium                   | About 0.5%.      |
| Beryllium                   | About 0.01%.     |
| Silicon                     | Up to 0.15% max. |
| Magnesium                   | The remainder.   |

2. Magnesium alloys as claimed in claim 1 in which the said lanthanum is utilized in the form of rare earths, containing up to substantially 4% neodymium and up to substantially 4% praseodymium, the remainder being lanthanum.

**References Cited in the file of this patent**

**UNITED STATES PATENTS**

|           |              |               |    |
|-----------|--------------|---------------|----|
| 1,941,039 | Luschenowsky | Dec. 26, 1933 | 10 |
| 2,302,968 | McDonald     | Nov. 24, 1942 |    |
| 2,420,293 | Bedk et al.  | May 13, 1947  |    |

|           |               |               |
|-----------|---------------|---------------|
| 2,549,955 | Jessup et al. | Apr. 24, 1951 |
| 2,569,477 | Leontis       | Oct. 2, 1951  |
| 2,609,309 | Meier         | Sept. 2, 1952 |
| 2,622,049 | Hesse         | Dec. 16, 1952 |

**FOREIGN PATENTS**

|               |                |
|---------------|----------------|
| Austria       | Sept. 18, 1941 |
| Great Britain | July 1, 1953   |

**OTHER REFERENCES**

Journal of Metals, vol. 1, pp. 968-983, December 1949.